

## UNITED STATES PATENT OFFICE

2,347,289

## PRINTING PROCESS

George W. Seymour, Cumberland, Md., assignor  
to Celanese Corporation of America, a corpora-  
tion of Delaware

No Drawing. Application October 14, 1940,  
Serial No. 361,103

## 6 Claims. (Cl. 8—64)

This invention relates to a process of dyeing fabrics, and relates more particularly to the application printing of fabrics by the use of printing paste compositions.

An object of my invention is the formulation of printing paste compositions which fully penetrate the fabrics upon which they are applied.

Another object of my invention is to obtain printed fabrics in which the designs are level in shade and free of mottling.

A further object of my invention is the formulation of printing paste compositions which are especially suitable for use with fabrics containing organic derivatives of cellulose.

Other objects of my invention will appear hereinafter from the following detailed description.

Printed textile fabrics in which the designs are composed of various colors have long been known to the art. These designs may be obtained in numerous ways. Generally, they are obtained by applying a printing paste composition to the fabrics whereby, depending upon the formulation of the printing paste composition, a variety of color effects may be obtained. Thus, fabric dyed in any suitable ground color may be printed in a particular pattern with a paste containing a discharging agent for the ground color. After the discharging action has been caused to take place by appropriate treatment of the printed fabric, a white pattern, where the paste has been applied, on a colored ground is obtained. If the paste contains a dyestuff together with the discharging agent an illuminated discharge is obtained, that is, one in which the discharged portion of the colored ground is colored by the dyestuff in the paste composition after the ground color has been destroyed by the discharge agent. Likewise, white fabrics may be printed in patterns of many colors by treating them with printing pastes containing various dyestuffs and applying these pastes in any desired pattern.

The discharge agents and the dyestuffs are generally applied to the fabrics in the form of a thick paste so that the area they cover may be controlled and the pattern in which they are printed may be accurately reproduced on the fabric. Various thickening and adhesive agents may be used in the formulation of the printing pastes and among the many agents which may be used are gum tragacanth, gum arabic, agar-agar, gum senegal, albumin, starch and British gums or dextrans. The British gums or dextrans are derived from starch. One method of preparing these gums is to thoroughly cook and hydrolyze it in enclosed chambers. Still another method comprises subjecting the starch to enzymatic action. The resulting products are known as British gums or dextrans and may differ somewhat in composition depending upon the

manner in which they are prepared. Ordinarily, they are complexes containing greater or lesser proportions of true dextrin, soluble starch, unaltered starch and glucose. The products are thick, gummy masses which have excellent adhesive properties and may be compounded or formulated into printing pastes by incorporating therein the desired dyestuffs, discharge agents and other desired inert or chemically active agents. While these pastes are suitable for the printing of light and loosely-woven fabrics, the results on heavier and more closely woven fabrics have not always been as even, as uniform or as deep in the fabric as desired.

I have now discovered that if the printing pastes are formulated using a gum base of incompletely hydrolyzed starches as the print paste thickener and adhesive, excellent and unusual penetration of the dyestuff into the fabric is obtained and the resulting prints are free of uneven, mottled or spotted areas.

Thus, the starch gums suitable for use in accordance with my invention may be prepared by incompletely hydrolyzing starch by heating the starch in water in the presence of a hydrolyzing catalyst such as hydrochloric, nitric or sulfuric acid. In order that the starch be incompletely hydrolyzed the conditions under which it is heated must be carefully controlled. The starch may be heated in water to temperatures of about 150° F. to 205° F. for periods of time ranging from 10 minutes to 4 hours. Where a catalyst such as nitric, sulfuric or hydrochloric acid is used to aid the hydrolysis, the mixture may be heated at reduced temperatures for shorter times. The amount of acid used will vary but in general from about 0.01% to 0.10% of concentrated acid based on the weight of the starch is sufficient to catalyze the hydrolysis so that when the starch is heated under the conditions described, the reaction will not be complete. Starches such as, for example, corn, rice, sago, potato, wheat, tapioca or cassava starch may be treated in accordance with my invention and excellent starch gums may be obtained.

In addition to the starch gum base and the dyestuffs, used in the formulation of the printing paste composition, other agents such as textile gum or other type of vegetable gum or British gum may be incorporated therein to give the resulting paste other desirable properties. In addition it is sometimes desirable to include organic water-soluble dyeing assistants which are for the most part solvents for the dyestuff. Assistants such as glycerol, glycols, etc., glycerol formals and other formals and "Glyezine A" (i. e. thiodiglycol) may be used.

The pastes may be applied to the fabric in the desired pattern in any suitable manner. They may be printed on by means of engraved or em-

bossed rolls, they may be brushed on, or else they may be sprayed on through stencils or screens.

While these printing pastes may be used for the printing of fabrics of cotton, silk, wool and the regenerated cellulose type of artificial fiber, they are especially suitable for the printing of fabrics made in whole or in part of organic derivatives of cellulose. Examples of organic derivatives of cellulose are cellulose esters such as cellulose acetate, cellulose propionate, cellulose butyrate and mixed esters such as cellulose acetate-propionate and cellulose acetate-butyrate, and organic ethers such as ethyl cellulose, methyl cellulose and benzyl cellulose. A mixed material may be one of cellulose acetate and cotton.

In order further to illustrate my invention but without being limited thereto the following example is given:

*Example*

300 parts of wheat starch are mixed with 1700 parts of water, heated to a temperature of about 175° F. and maintained at approximately that temperature for about 2 hours. The starch is unboiled and is partially but incompletely hydrolyzed by this treatment and is left in a thick gummy mass.

A printing paste consisting of:

| Parts                                                         |     |
|---------------------------------------------------------------|-----|
| Celliton Fast Pink FF3B, 25% ground in commercial British gum | 100 |
| Wheat starch paste prepared as above                          | 400 |
| Water                                                         | 500 |

is thoroughly mixed to a smooth homogeneous mass and applied to a cellulose acetate fabric of heavy sharkskin weave by means of engraved rolls. The printed fabric is dried and then passed through a suitable ager where it is subjected to the action of wet steam under 5 lbs. pressure for about 15 minutes. The fabric is then lightly soaped and finished as required, yielding a red print on a white background.

Alternatively, a somewhat thicker printing paste may be used consisting of:

| Parts                                                                                                |     |
|------------------------------------------------------------------------------------------------------|-----|
| Celliton Fast Pink FF3B (Schultz, Second Supplement, page 142), 25% ground in commercial British gum | 100 |
| Wheat starch paste                                                                                   | 700 |
| Water                                                                                                | 200 |

It is to be understood that the foregoing detailed description is given merely by way of illus-

tration and that many variations may be made therein without departing from the spirit of my invention.

Having described my invention, what I desire to secure by Letters Patent is:

- 5 1. In the process of producing local color effects upon textile materials, the step of locally applying thereto a paste comprising a substance capable of effecting color change and, as thickening component, starch that has been heated in water containing at most 0.10% of mineral acid based on the weight of the starch at a temperature of 150 to 205° F. for from 4 hours to 10 minutes.
- 10 15 2. In the process of producing local color effects upon textile materials containing cellulose acetate yarns, the step of locally applying there a paste comprising a substance capable of effecting color change and, as thickening component, starch that has been heated in water containing at most 0.10% of mineral acid based on the weight of the starch at a temperature of 150 to 205° F. for from 4 hours to 10 minutes.
- 20 25 3. In the process of producing local color effects upon textile materials, the step of locally applying thereto a paste comprising a substance capable of effecting color change and, as thickening component, starch that has been heated in water alone at a temperature of 150 to 205° F. for from 4 hours to 10 minutes.
- 30 35 4. In the process of producing local color effects upon textile materials containing cellulose acetate yarns, the step of locally applying thereto a paste comprising a substance capable of effecting color change and, as thickening component, starch that has been heated in water alone at a temperature of 150 to 205° F. for from 4 hours to 10 minutes.
- 40 45 5. A printing composition for application to textile materials comprising a substance capable of effecting color change and, as thickening component, starch that has been heated in water containing at most 0.10% of mineral acid based on the weight of the starch at a temperature of 150 to 205° F. for from 4 hours to 10 minutes.
- 50 6. A printing composition for application to textile materials comprising a substance capable of effecting color change and, as thickening component, starch that has been heated in water alone at a temperature of 150 to 205° F. for from 4 hours to 10 minutes.

GEORGE W. SEYMOUR.